

## UNITED STATES PATENT OFFICE.

VIKTOR BÖHM, OF VIENNA, AUSTRIA.

## PROCESS FOR CARROTING ANIMAL FIBERS.

No Drawing. Application filed October 1, 1925, Serial No. 59,973, and in Austria November 20, 1924.

This invention relates to the working up of animal fibers, such for example as hair, into felts, more particularly for the manufacture of hats.

5 The invention is based on the discovery that by treating animal fibers, such for example as the hair of hares, rabbits or the like, with aldehyde and ketone carroting means, felts of high value are obtainable, and that 10 by secretages of this kind a refinement or improvement of the fibers or hair is effected, whereby on the one hand its felting or fulling properties amongst other things are enhanced and its yield is increased, and on the 15 other hand even inferior sorts of fiber or hair are materially improved in quality. Waste hair and even long coarse hair as distinguished from wool hair which is subjected to the process according to the invention 20 assumes properties which enable it to be completely utilized for the manufacture of hat bodies or foundations without leading to inferior products.

The process according to the invention 25 however also enables waste from other industries, such for example as waste and hair arising from tanning and fur industries, to be rendered usable for the manufacture of hat bodies.

30 The aldehyde and ketone carroting means may be employed either alone or in conjunction with other carroting means, such for example as metallic salt secretages such as mercury secretages and the like.

35 Amongst aldehyde carroting means there are to be considered carroting means which contain formaldehyde, acetaldehyde, benzaldehyde and the like, singly or mixed together, and also their compounds, more particularly 40 with bisulphites or which consist of or decompose into these materials, particularly formaldehyde. As aldehyde mixtures there are for example also available the aldehydes obtained from the fusel oil spirit manufacture, as obtained chiefly from the first runnings.

45 Amongst ketone carroting means are to be considered carroting means containing acetone, aceto-acetic ester, acetophenone and the like, and also their compounds or mixtures, consisting of these materials or decomposing into them.

50 These secretages, such for example as formaldehyde, may also be utilized in the form of vapour.

The aldehyde and ketone carroting means

according to the invention enable carroting by laying the hair therein, in which case both the skin and also loose hairs can be subjected to such a carroting or secretage process. 60

To the carroting process according to the invention may also be subjected fur the felting of which has been begun in the ordinary way, or half-planked or sized felt (Labraz) or this carroting means may be added to the 65 planking or sizing liquid and the planking or felting properties of the fur or half-planked felt thereby materially improved.

After the secretage process, a treatment 70 with an oxidizing medium, such for example as hydrogen peroxide, a permanganate, a perborate or the like is preferable, whereby the unpleasant smell of the aldehydes or ketones can be taken from the carroted goods. The use of an oxidizing medium which enhances the carroting effect is preferable, such 75 for example, as hydrogen peroxide, nitric acid or the like.

## Example.

80 The hair of hares, rabbits or the like is placed in a formaldehyde solution of any desired concentration or dilution, slightly acidified with sulphuric acid, hydrochloric acid or the like, and exposed to the action of 85 this solution at a raised temperature between about 25° and 80° centigrade. The duration of the reaction varies according to the quality of the hair and the concentration and temperature of the solution from half an hour 90 to 40 hours or more. Hereupon it is drained or centrifuged and then treated with an oxidizing medium such as hydrogen peroxide, whereby the unpleasant smell of the formaldehyde is eliminated. 95

The process according to the invention may also be carried out under pressure at temperatures above 100° C.

Furthermore the process can also be carried out by exposing the hair, moistened if 100 desired with water, to formaldehyde vapours.

Aldehydes and ketones have in common the feature nicely distinguishing them from any other organic compounds, that they contain one or more carbonyl (C=O) groups. 105

## What I claim is:

1. The process of treating animal fibers comprising carroting said fibers by treating them with a neutral carroting agent containing a carbonyl group. 110
2. The process of treating animal fibers comprising carroting said fibers by subject-

- ing them to the action of a carrottting agent comprising formaldehyde.
3. The process of treating animal fibers comprising felting said fibers and during 5 said felting treating said fibers with a neutral carrottting agent containing a carbonyl group.
4. The process of treating animal fibers which comprises carrottting said fibers by 10 treating them with a neutral carrottting agent containing a carbonyl group and treating
- said carrottted fibers with an oxidizing medium.
5. A process for treating animal fibers comprising carrottting said fibers by treating 15 them with a carrottting agent containing substances which on decomposition yield a neutral carrottting agent containing a carbonyl group.

In witness whereof I have hereunto signed 20 my name.

VIKTOR BÖHM.